

## UNITED STATES PATENT OFFICE

JOHN STROTHER MILLER, JR., OF RAHWAY, NEW JERSEY, ASSIGNOR TO THE BARBER ASPHALT COMPANY, OF PHILADELPHIA, PENNSYLVANIA, A CORPORATION OF WEST VIRGINIA

## MANUFACTURE OF BITUMINOUS EMULSIONS

No Drawing.

Application filed July 17, 1920. Serial No. 397,027.

My invention relates to bituminous emulsions for suspensions and their manufacture, and is especially concerned with the emulsification of relatively hard bitumens and bituminous materials solid at ordinary temperatures. For convenience, I have herein-after referred to bitumens and bituminous materials generally as "bituminous bases," or, still more briefly, as "bases." 10 The common commercial processes of aqueously emulsifying bituminous bases involve direct and intimate intermixture of the base in a sufficiently fluid state with water. In many or most cases, this requires that both 15 the base and the water be heated; the base to render it sufficiently fluid, and the water in order that the attempted intermixture may not chill the base so much as to render emulsive combination impossible. To avoid chilling troubles, therefore, the water must be raised as nearly as possible to the temperature of the base when fluid; so that the application of this process of emulsifying by direct fluid intermixture is limited to bases 20 of not more than moderate hardness at ordinary temperatures. Solid bituminous bases of consistency harder than 30 mm. when tested with a standard Roberts-Sharp #2 needle under a load of 100 grammes acting for 25 5 seconds at 77° F. (according to the standard method of the American Society for Testing Materials) have generally proved impractical 30 of emulsification by such a process. Accordingly, the native asphalts generally are 35 emulsified by direct fluid intermixture only after having been suitably softened by "fluxing" with mineral oils or the like, and the artificial or "oil" asphalts only when similarly 40 softened, or when themselves of proper consistency at moderate temperatures.

There has, indeed, been proposed a somewhat indirect process of emulsification, by fluid intermixture with the aid of organic solvents; and even relatively hard solid bases have been thus treated. This indirect process is, however, somewhat complicated, costly, and unsatisfactory,—owing, in part, to the operations necessary for the recovery of the 45 solvent used. Moreover, its application is

necessarily limited to the bases for which suitable solvents are commercially available.

My invention makes it possible to emulsify solid bituminous bases,—whether natural or artificial, and whether simple, fluxed, or otherwise composite,—without the aid of solvents, and without necessity of softening them by heat. Such emulsification can be effected without dependence upon heat, I have discovered, by bringing the solid base into intermixture with the desired liquid medium while or after reducing it to a suitably fine state of division—all at ordinary temperatures or "in the cold." The bituminous dispersion or suspension produced by this process of direct solid and fluid intermixture in the cold has all the useful properties of so-called bituminous emulsions of the prior art produced by direct fluid intermixture with the aid of heat, and may, therefore, fairly be regarded as an emulsion. And even though the bituminous particles of this dispersion or suspension be not in the globular fluid state characteristic of emulsions strictu sensu, yet since many of the bases heretofore emulsified by direct fluid intermixture with the aid of heat are solid when cold, it would appear that in all probability the suspended bituminous globules of their emulsions so produced are solid rather than liquid after cooling of the emulsion, and that my products are emulsions in the same sense that they are. 70

Aqueous emulsions of solid natural or artificial bituminous bases, and more particularly emulsions of solid asphaltum bases, as native asphalt, gilsonite, petroleum still residues, and the like, may be prepared on this principle with mechanical reduction of the base in its solid state to a finely divided condition, by grinding, mixing, and emulsively combining the base (either crude or refined) with water in the presence of an emulsifying or peptonizing material or agent, prone to or promotive of emulsification,—such as soap, starch, finely divided mineral or inorganic material like clay, etc. Natural asphalts ordinarily requiring to be refined (such as Trinidad Lake, Bermudez Lake, Maracaibo, etc.) may be thus finely ground 85 unrefined, or in their crude native state, in 90

the presence of water and emulsifying agent. In thus emulsifying such natural asphalts unrefined, due allowance for their natural water content should be made in adding water to give the amount desired in the final product; while in emulsifying refined natural asphalts, artificial asphalts, tar, and other water-free bituminous bases, the full amount of water desired must be added.

16 Bituminous emulsions prepared by such direct intermixture with mechanical division differ from those prepared with the aid of heat in the roughness, irregularity, and angularity of their suspended finely divided 17 or ground particles as contrasted with the smooth roundness of solidified globules of liquid base. Such roughness and irregularity tend to greater resistance of the particles against "settling" out or "breaking" of the 20 emulsion, so that the emulsion thus produced is essentially a new manufacture, and thoroughly stable. The particles are in a colloidal or semi-colloidal state of fineness and thoroughly deflocculated, so that they do not 25 tend to adhere together until or unless the emulsion is dried or otherwise broken. The emulsion is "creamy" in appearance and feel, not at all sandy.

In contrast to artificial bitumens like coal- 30 tar pitch or water-gas pitch, certain hard natural bitumens or bases in their native state show emulsification or emulsifying properties (or both) in greater or less degree,—either by reason of emulsive combination in 35 them of a water content that gives them somewhat the character of "solid emulsions," or by reason of the presence in them, as impurity, of material having emulsifying properties. Such natural bitumens, I have dis- 40 covered, may be emulsified by being finely ground in the presence of water without the addition of any foreign emulsifying agent, or with a less addition than would otherwise be required. An example of such a natural 45 self emulsifying base is crude Trinidad Lake asphalt, which contains emulsiuent finely di- 50 vided inorganic material of clayey character that acts as an emulsifying agent when the base is ground as hereinbefore mentioned, as well as some emulsively combined "native" water.

My invention, it will be seen, not only serves for the emulsification of even the hardest bituminous bases by and of them- 55 selves, but also affords a means of producing useful emulsion compositions or combinations of ingredients that could not readily be incorporated together in the way of fluxing, or of hard and soft bituminous components 60 generally. When such emulsion combinations of hard and soft bases are desired, the hard base may be ground and mixed, in the presence of an emulsifying agent, with water and emulsively suspended soft base. The 65 grinding of the hard base in the presence of

an emulsifying agent and its mixture with water and with emulsively suspended soft base need not necessarily be performed as separate operations, but may be effected in one single operation, by simply grinding the hard base with soft base emulsion containing sufficient water to form a final composite product with the desired aqueous content.

For the benefit of those desiring to practice my invention, I will now describe, by way of example, the manufacture of a typical emulsion of Trinidad Lake asphalt, the proportions mentioned being by weight:

|                             | Parts |
|-----------------------------|-------|
| Crude Trinidad Lake asphalt | 57    |
| Water                       | 29    |
| Rosin oil soda soap         | 5     |

The hard base should first be broken or crushed (coarsely ground) into conveniently small fragments and grains; it should then be ground with the water and the soap in a ball-mill until the bituminous mass becomes thoroughly homogeneous, when the finely ground base will be found to have become thoroughly intermixed and emulsively combined with the water and the emulsifying agent. The resultant product has the useful properties characteristic of bituminous emulsions generally, with the special advantages due to the hardness of its bituminous content.

The total amount of soap or other emulsifying material (whether foreign like soap, or of a character native to the bitumen, like the clay of Trinidad Lake asphalt) that should be present is subject, of course, to considerable variation, according to the stability of the product desired under all conditions of thinning with water. The thinner the emulsion it is desired to produce (either initially or by subsequent thinning for use), the higher the proportion of soap to bituminous base should be. The proportions indicated are about right for good economy, and will insure a product sufficiently liquid to flow readily.

The bituminous emulsion produced as just described is suitable and desirable for various special purposes,—such as flooring mixtures, mastic mixture for vertical walls, and for some forms of water-proofing, etc. For many purposes, indeed, its bituminous content is too hard; but this can readily be softened by admixture or intermixture of "soft" bituminous emulsion (made with a relatively soft base by any known or preferred process) with the "hard" emulsion, according to the methods indicated above. Soft base emulsions can be very readily made from liquid petroleum fluxes by methods well known to the art; and by proper mixing of such emulsified flux or the like with my hard base emulsion, the consistency of the total base or residue of the emulsion combination can be varied at will from that of the hard base to that of

the liquid petroleum flux. These soft and hard base emulsion combinations are of very general and varied utility,—as distinguished from the limited and special utility of hard emulsions referred to above,—by reason of this flexibility of control over the consistency of their total base content or residue, and can be adapted and employed for almost any purpose for which bituminous materials are useful.

Having thus described my invention, I claim:

1. The process of preparing an aqueous emulsion of natural solid bituminous base self-emulsifying by reason of native impurity which consists in finely grinding such base, in its solid native state, with water and continuing the grinding until a water external phase emulsive combination is effected.

2. The process of preparing an aqueous emulsion of natural solid bituminous base natively containing emulsifying finely divided material which consists in mechanically reducing the base in its solid native state to a condition of fine division in the presence of water and intimately mixing the solid base thus finely divided with the water until a water external phase emulsive combination is effected.

3. The process of preparing aqueous emulsion combinations of hard and soft asphaltum bases which consists in finely grinding the hard base and mixing the same, in the presence of an emulsifying agent and in the solid state, with water and with emulsively suspended soft base.

4. As a new manufacture, fluid aqueous bituminous emulsion comprising hard natural asphaltum base in the solid state, finely ground and emulsively combined with water and a native content of emulsifying finely divided material with water in the external phase.

5. As a manufacture, an aqueous bituminous emulsion comprising finely ground hard asphaltum base in the solid state, mixed and emulsively combined with water and with emulsively suspended soft bituminous base with water in the external phase.

6. The process of preparing a thoroughly stable fluid emulsion from a solid asphaltum base by direct intermixture in the cold of such base with a desired liquid medium, which includes grinding a solid asphaltum base to a degree of fineness at which it will emulsively combine with a desired liquid medium in a solid state and without dependence upon heat and effecting an emulsive combination of the finely ground base with a desired liquid medium in external phase in the presence of an emulsifying material.

7. The process of preparing a thoroughly stable fluid emulsion from a solid asphaltum base by direct intermixture in the cold of such base with water, which includes grind-

ing a solid asphaltum base in the presence of water to a degree of fineness at which it will emulsively combine with the water in a solid state without dependence upon heat and continuing the grinding in the presence of an emulsifying material to effect an emulsive combination of the base and the water with the water in external phase.

8. The process of preparing a thoroughly stable fluid emulsion from a solid asphaltum base by direct intermixture in the cold of such base with water, which includes grinding a solid asphaltum base in the presence of water to a degree of fineness at which it will emulsively combine with the water in a solid state without dependence upon heat and continuing the grinding in the presence of finely divided inorganic emulsifying material to effect an emulsive combination of the base and the water with the water in external phase.

9. As a new article of manufacture a fluid aqueous bituminous emulsion comprising a finely ground asphaltum base the particles of which are emulsively combined in the solid state with water and emulsifying material, the water being in external phase.

10. The process of preparing an emulsive combination of a non-fluid asphaltum, which includes grinding a non-fluid asphaltum with a liquid medium containing a protective colloid until the asphaltum reaches a degree of fineness such as to emulsively combine with the liquid medium.

In testimony whereof, I have hereunto signed my name at Maurer, N. J., this 15th day of July, 1920.

JOHN STROTHER MILLER, JR.

70

75

80

85

90

95

100

105

110

115

120

125

130